# EUROPEAN PATENT SPECIFICATION

(11) **EP 2 473 655 B1**
(45) Date of publication and mention of the grant of the patent: **04.09.2013**
(21) Application number: 10731801.6
(22) Date of filing: 18.06.2010
(51) Int. Cl.: D01D 5/253, E01C 13/08

(54) **FIBER FOR ARTIFICIAL TURF**
KUNSTRASENFASER
FIBRE DE GAZON ARTIFICIEL

(30) Priority: 03.09.2009 ES 200930645
(43) Date of publication of application: 11.07.2012
(73) Proprietor: Mondo S.p.A., 12051 Alba Frazione Gallo (CN) (IT)
(72) Inventor: TESTA, Emanuele, I-12051 Alba Frazione Gallo (Cuneo) (IT)
(74) Representative: Frontoni, Stefano
(86) International application number: PCT/IB2010/052761
(87) International publication number: WO 2011/027235

(56) References cited:
- EP-A1- 0 648 868
- WO-A2-2005/005731
- GB-A- 1 166 361
- JP-A- 2007 277 739
- KR-A- 20090 041 781
- US-A- 3 837 980
- US-A- 3 940 522

## Description

### OBJECT OF THE INVENTION

The following invention, according to what is expressed in the statement of the present specification, relates to a fiber for artificial turf, being of the type of fibers utilized in the manufacturing of artificial turf carpets, by weaving the fibers, such that the essential object is to obtain a fiber with some resilient characteristics which make it recover its vertical position after being compressed, occasionally or temporarily, maintaining its original appearance for a long time.

For that purpose, the extruded monofilament fiber manufactured with polyolefins in polyethylene, has a certain cross section, and the height of the fibers forming the turf carpets present a certain length.

In this manner, the fibers forming the artificial turf carpet are allowed to recover their vertical position after being subjected to successive loads.

### FIELD OF APPLICATION

In the present specification, a fiber for artificial turf is described, of special application in manufacturing artificial fiber carpets for turf in the installation of fields for different sports, such as soccer, golf, rugby, or hockey.

In the same way, the fiber for artificial turf is equally applied to other uses, such as gardens, access roads, or decoration.

### BACKGROUND OF THE INVENTION

As it is known, each day there are more organizations and sports clubs opting to provide their installations, with playing fields for different sports, with artificial turf as an alternative to natural grass turf since they require less maintenance and to offer a sensation similar to the one of natural grass turf and to present improvements, such as, an artificial turf field can be used all year round, and the natural grass turf fields by requiring a recovery period in which they cannot be used. These artificial turf carpets are manufactured by weaving the artificial fibers.

On the other hand, with the object to obtain artificial turf carpets with fibers that maintain their characteristics over time, the monofilament fibers should have high resilience which makes them recover their vertical position after having been occasionally or temporarily compressed over time, preventing the fibers staying tilted over the ground.

In this manner, it has been attempted to obtain fibers made of different materials and sections with the object to provide them with high resilience, being able to consider the patent documents US 6,432,505; EP 1837423, and PCT W02005/005731.

In this way, in the American patent US 6,432,505, a synthetic turf is described having a substrate and a plurality of turf filaments made of synthetic polymer anchored to the substrate, said filaments having a diamond-shaped cross section, with a longitudinal axis along from one end to another end, and a lateral axis located in the middle, so that the thickness of the filament gradually decreases from said lateral axis, substantially, symmetrically and smoothly over the longitudinal axis toward each end.

In the European patent EP 1837423, a synthetic turf is described comprising a turf carpet and some knots projecting therefrom, the knots comprise individual filament strands and at least one shredded strand and, at least, a number of said strands consists essentially of a mixture of high density polyethylene and low density linear polyethylene.

In the patent PCT W02005/005731, an artificial turf filament is described wherein the filament has, in cross section, a central area and two wing areas in the opposite sides of said central area, and with a divergent orientation, such that an outward protruding head is formed at one side of the divergent areas of the central area, and at the far side from the divergent areas, the central area, has a face which is essentially aligned in the place of said central area and which is merged to the adjacent faces of each wing area.

### DESCRIPTION OF THE INVENTION

In the present specification, a fiber for artificial turf is described, being of the type of monofilament fibers utilized in the manufacturing of artificial turf carpets, by weaving the fibers and which are obtained by extrusion in polyethylene or another material, such that the fiber for artificial turf presents a flat rectangular cross section with its shorter sides rounded, in the central part of one of its longer faces being provided with a curved-convex projection, and in its other longer face is provided with a pair of projections, equally curved-convex, in a symmetrical position with respect to its central axis.

In a preferred embodiment, the fiber for artificial turf has a width of approximately 1400 µm.

In the same way, in a preferred implementation the fibers for artificial turf which form the carpets have a height of approximately 60 mm.

The thickness of the fiber for artificial turf in the central part of the curved-convex projections is the same for all of them, such that in a preferred implementation the thickness of the fiber for artificial turf in the central part of the curved-convex projections is of approximately 270 µm.

For supplementing the description to be carried out next, and with the object to aid to a better understanding of the characteristics of the invention, a set of drawings is attached to the present specification, with figures where the most characteristic details of the invention are depicted in an illustrative but not limitative manner.

### BRIEF DESCRIPTION OF THE DESIGNS

Figure 1. Shows a perspective view of a segment of a fiber for artificial turf, being able to observe the cross section thereof.
Figure 2. Shows a detailed perspective view of some weaved fibers forming the corresponding carpet for artificial turf.
Figure 3. Shows a results table of the recovery index of the fibers, with different cross sections, to be analyzed, with a height of 60 mm, according to the elapsed time of 1, 30 and 240 minutes from its release from a compressive load.
Figure 4. Shows an evolution table of the fibers in their recovery over time of 1, 30 and 240 minutes after their release from a compressive load, according to the recovery index of the analyzed fibers with a height of 60 mm.
Figure 5.- Shows a classification table of the analyzed fibers according to a height of 60 mm, according to the elapsed time of 1, 30 and 240 minutes, after their release from a compressive load.

### DESCRIPTION OF A PREFERRED EMBODIMENT

Given that the resilience of the fibers forming the carpets for artificial turf is affected by both their section and the height of the fibers forming them, with the object to obtain a fiber for artificial turf with high resilience which facilitates its recovery against successive occasional or temporary loads and maintains its original appearance, a series of samples of fibers of different sections have been analyzed in order to obtain that fiber presenting higher resilience.

In this way, taking into account that both the height of the fibers forming the carpets for artificial turf and its section affect the recovery thereof, i.e. their resilience and utilizing the method described in the Patent of Invention P200930107 wherein a *method for determining the recovery grade in artificial fiber carpets* is described, an analysis has been carried out in order to assess the recovery of fibers with different sections, for which it determines the recovery index as well as the recovery rate, such that this parameter points out the speed at which a material recovers after being released from a load.

From these premises, four samples of artificial turf carpets have been analyzed, with fibers of different sections being manufactured from monofilament extruded polyethylene, and the fibers forming the carpets have a height of 60 mm, one of the samples being the fiber object of the invention with a certain section which confers it high resilience.

In this way, the section of the fiber object of the invention has been subjected to an analysis together with three more samples of different sections, so that the cross section of the fiber 1 object of the invention (corresponding to the sample of section 3) presents a flat rectangular general shape with its shorter sides rounded, in the central part of one of its longer faces being provided with a curved-convex projection 2, and in its other longer face is provided with a pair of curved-convex projections 3 in a symmetrical position with respect to its central axis.

In this manner, the special section of the sample 3 based on the curved-convex projections of its longer faces confer it with high resilience, in which the height of the fiber forming the artificial turf carpets collaborates.

Moreover, in a preferred implementation of the fiber 1 for forming artificial turf carpets, it has a width "D" of approximately 1400 µm.

On the other hand, the thickness "d" of the fiber for artificial turf in the central part of the curved-convex projections is the same in all of them, such that in a preferred implementation is of approximately 270 µm.

In this way, as observed in figure 2 of the designs, fibers 1 forming the weaved bundles of the artificial turf carpet, will have a height preferably of 60 mm, although, logically, the height could be another one.

As in the cited patent P200930107, the method is specified based on applying to the samples a constant compressive load of 1400 kg during 72 hours, such that, once said time is elapsed, the load is released and images of the same zone are captured after 1, 30 and 240 minutes. Before applying the compressive load, an image has also been taken in order to know and define the total area occupied by the fibers, this value corresponding to 100% of the fibers in their state of equilibrium.

The captured images are analyzed for each one of the times and the area occupied by the fibers is calculated, assigning 100% recovery to the initial area occupied by the fibers before applying the load, such that calculating the recovery index is carried out applying the following ratio $Recovery index \left(%\right) ,$

In this way, applying the described methodology, the results of the recovery index have been obtained for the carpets formed of some fibers with a height of 60 mm, shown in the table of figure 3, after a time of 1, 30 and 240 minutes of being released from the load, being able to observe how the sample of section 3 presents a recovery index of 100% already at 30 minutes of releasing the load.

In the same way, in figure 3 of the designs, the evolution of the recovery index is observed in the four analyzed samples at a fiber height of 60 mm, so that once the stationary time (240 minutes) is reached, the recovery considerably increases arriving, in the samples object of the invention, to said value.

In figure 4 of the designs, the classification of the result obtained from the four analyzed samples is depicted, being able to observe how the fibers of the sample 3 object of the invention are the ones that recover more, having logically, higher resilience.

Lastly, in figure 5 of the designs the evolution of the recovery index of the four analyzed samples is depicted at a fiber height of 60 mm, being able to observe how the sample 3 object of the invention is the one having a greater recovery index.

In this manner, it is concluded that a fiber 1 for forming carpets for artificial turf with a flat rectangular general cross section with its shorter sides rounded, and in the central part of its longer faces provided with a curved-convex projection 2, and in its other longer face provided with a pair of curved-convex projections 3 in a symmetrical position with respect to its central axis, presents high resilience making the fibers forming the artificial turf carpets to recover their vertical position after being subjected to some successive compressive loads and making them to maintain their original aesthetics over time.

In a preferred implementation of the fiber 1 for forming artificial turf carpets, it has a width "D" of approximately 1400 µm.

On the other hand, the thickness "d" of the fiber for artificial turf in the central part of the curved-convex projections is the same for all of them, such that in a preferred implementation is of approximately 270 µm.

## Claims

1. FIBER FOR ARTIFICIAL TURF, being of the type of monofilament fibers utilized in the manufacturing of artificial turf carpets and which are obtained by extrusion in polyethylene or another material, **characterized in that** the fiber (1) forming the carpets for artificial turf presents a flat rectangular general cross section with its shorter sides rounded, in the central part of one of its longer faces being provided with a curved-convex projection (2), and in its other longer face provided with a pair of curved-convex projections (3) in a symmetrical position with respect to its central axis.

2. FIBER FOR ARTIFICIAL TURF, according to claim 1, **characterized in that** the fiber (1) forming the carpets for artificial turf has a height of approximately 60 mm.

3. FIBER FOR ARTIFICIAL TURF, according to claim 1, **characterized in that** the fiber (1) forming the carpets for artificial turf has a width of approximately 1400 µm.

4. FIBER FOR ARTIFICIAL TURF, according to claim 1, **characterized in that** the thickness of the fiber (1) forming the carpets for artificial turf in the central part of the curved-convex projections is the same for all of them.

5. FIBER FOR ARTIFICIAL TURF, according to claims 1 and 4, **characterized in that** the thickness of the fiber (1) forming the carpets for artificial turf in the central part of the curved-convex projections is of approximately 270 µm.

## Patentansprüche

1. Kunstrasenfaser eines Typs von Monofilfasern, die bei der Herstellung von Kunstrasenteppichen verwendet werden und die man durch Extrudieren von Polyethylen oder einem anderen Material erhält, **dadurch gekennzeichnet, dass** die Faser (1), die die Kunstrasenteppiche ausbildet, einen im wesentlichen flachen rechteckigen Querschnitt aufweist, dessen kürzere Seiten abgerundet sind, sich in dem zentralen Teil einer seiner längeren Flächen ein gekrümmter konvexer Vorsprung (2) befindet und seine andere längere Fläche mit zwei gekrümmten konvexen Vorsprüngen (3) in einer symmetrischen Position in Bezug auf dessen Mittelachse versehen ist.

2. Kunstrasenfaser nach Anspruch 1, **dadurch gekennzeichnet, dass** die Faser (1), die die Kunstrasenteppiche ausbildet, eine Höhe von etwa 60 mm hat.

3. Kunstrasenfaser nach Anspruch 1, **dadurch gekennzeichnet, dass** die Faser (1), die die Kunstrasenteppiche ausbildet, eine Breite von etwa 1.400 µm hat.

4. Kunstrasenfaser nach Anspruch 1, **dadurch gekennzeichnet, dass** die Dicke der Faser (1), die die Kunstrasenteppiche ausbildet, in dem zentralen Teil der gekrümmten konvexen Vorsprünge für sämtliche Fasern dieselbe ist.

5. Kunstrasenfaser nach Anspruch 1 und 4, **dadurch gekennzeichnet, dass** die Dicke der Faser (1), die die Kunstrasenteppiche ausbildet, in dem zentralen Teil der gekrümmten konvexen Vorsprünge etwa 270 µm beträgt.

## Revendications

1. Fibre pour gazon artificiel, du type fibres monofilaments utilisées pour la fabrication de tapis de gazon artificiel et qui sont obtenues par extrusion de polyéthylène ou d'un autre matériau, **caractérisée en ce que** la fibre (1) formant les tapis pour le gazon artificiel présente une section transversale générale rectangulaire plate avec ses côtés plus courts arrondis, une protubérance incurvée convexe (2) étant prévue dans la partie centrale de l'une de ses faces plus longues, et une paire de protubérances incurvées convexes (3) étant prévues dans son autre face plus longue à une position symétrique par rapport son axe central.

2. Fibre pour gazon artificiel, selon la revendication 1, **caractérisée en ce que** la fibre (1) formant les tapis pour le gazon artificiel a une hauteur d'environ 60 mm.

3. Fibre pour gazon artificiel, selon la revendication 1, **caractérisée en ce que** la fibre (1) formant les tapis pour le gazon artificiel a une largeur d'environ 1400 µm.

4. Fibre pour gazon artificiel, selon la revendication 1, **caractérisée en ce que** l'épaisseur de la fibre (1) formant les tapis pour le gazon artificiel dans la partie centrale des protubérances incurvées convexes est la même pour la totalité de celles-ci.

5. Fibre pour gazon artificiel, selon les revendications 1 et 4, **caractérisée en ce que** l'épaisseur de la fibre (1) formant les tapis pour le gazon artificiel dans la partie centrale des protubérances incurvées convexes est d'environ 270 µm.
